# EUROPEAN PATENT SPECIFICATION

(11) **EP 0 342 408 B1**
(45) Date of publication and mention of the grant of the patent: **11.08.1993**
(21) Application number: 89107705.9
(22) Date of filing: 27.04.1989
(51) Int. Cl.: B21B 45/02, B21B 15/00, B21B 27/00, B21H 8/00, B21H 7/00

(54) **Rolling method and rolling machine**
Walzverfahren und Walzwerk
Procédé de laminage et train de laminage

(30) Priority: 18.05.1988 JP 119313/88
(43) Date of publication of application: 23.11.1989
(73) Proprietor: MITSUBISHI JUKOGYO KABUSHIKI KAISHA, Tokyo 100 (JP)
(72) Inventor: Mito, Yoshiki Hiroshima Mach. Works Mitsubishi, Nishi-ku Hiroshima-shi Hiroshima-ken (JP); Aratani, Hiroshi Hiroshima Mach. Works Mitsubishi, Nishi-ku Hiroshima-shi Hiroshima-ken (JP); Morimoto, Kazuo Hiroshima Mach. Works Mitsubishi, Nishi-ku Hiroshima-shi Hiroshima-ken (JP)
(74) Representative: Henkel, Feiler, Hänzel & Partner

(56) References cited:
- WO-A-82/03575
- DE-C- 635 220
- FR-A- 2 290 623
- US-A- 1 490 944
- US-A- 1 960 958
- US-A- 2 361 039

## Description

This invention relates to a method and a machine for rolling metal plate, shape steel, bar steel, etc. made of steel, aluminum and the like with a reduced coefficient of friction.

In rolling a band plate made of steel, aluminum and the like, nowadays, a hot strip mill is used in case of hot rolling, or a tandem cold mill is used in case of cold rolling, for example. In such mills, the band plate is rolled thin by putting it between a pair of upper and lower rotating work rolls. To reduce the friction arising between the work roll and the band plate when the rolling takes place, hitherto, fluid such as a rolling lubricating agent was supplied to the surface of the work roll to decrease a load devoted to causing plastic deformation. In this regard, the lubricating agent is effective in preventing the generation of abrasion of the work roll and of flaws in the surface of a workpiece to be rolled.

In case of hot rolling, however, the temperature of the band plate reaches about 900°C to 1200°C, and the rolling lubricating agent supplied to the work roll loses its lubricating power because it generally burns at temperatures above 200°C. Consequently, the rolling lubricating agent adhering to part of the work roll exerts only a poor lubrication effect, thereby increasing the abrasion of the roll. With an increase in abrasion of the roll, the coefficient of friction between the band plate and the roll increases; hence, a large rolling load must be imposed to keep the reduction ratio of the band plate.

According to the conventional hot rolling process, there is no fluid, but air present between the work roll and the band plate, and the air cannot contribute as a boundary film because of its compressibility, thus, it is deemed that every surface region of the band plate is brought into a boundary friction state wherein metal-to-metal contact prevails. Therefore, the coefficient of friction between the work roll and the band plate becomes 0.2 or more (µ ≧ 0.2); consequently, the rolling load increases, the surface of the roll becomes rough, the roll wears, and so on.

As a result, the rolled band plate has surface irregularity in the widthwise direction, such as local projection or high spot, defective shape, and zigzag pattern.

In case of cold rolling, to increase the reduction ratio, the pressure within the contacting arc region between the band plate and the work roll for rolling the former is made very high; thus, the rolling lubricating agent cannot get enough into the contacting arc region of the roll to thereby exert only a poor lubrication effect.

DE-C-635220 discloses a method according to the pre-characterising part of claim 1 to mechanically or chemically pretreat a workpiece in order to obtain a roughened surface. Thereafter, the workpiece is covered with a liquid containing solid and/or organic compounds. After a drying period of approximately 15 minutes, a solidified coating covers the workpiece. The compounds or particles contained in the liquid are supposed to intrude into the rough surface of the workpiece and to provide an intimate contact with the surface that cannot be wiped off too easily. After this coating of the workpiece, it is cold rolled.

US-A-1.490.944 discloses a hot rolling mill according to the pre-characterising part of claim 2 having a rough-rolling section and a smooth rolling section. In the first station pockets are formed into the surface of the workpiece which is washed with water beneath the pocket-forming roll.

In view of the foregoing circumstances, it is the object of the present invention to provide a rolling method as described in the opening clause of claim 1 and rolling machine capable of reducing the abrasion of rolls of a rolling mill, decreasing the rolling load, keeping the reduction ration identical with the prior art, and making the rolling machine compact.

To achieve the foregoing object, the above described rolling method is characterized by the steps of claim 1.

In operation, a large number of recesses are formed in the surface of a workpiece to be rolled by the recess impressing unit provided on the inlet side of the rolling mill, then, at the time of rolling the workpiece by the rolling mill, a lubricating fluid is retained and confined in the recesses, and when the workpiece is pressed, the lubricating fluid thus confined is expanded thin to form a boundary film. It should be noted that the recesses disappear as the rolling of the workpiece progresses, and the surface of the workpiece after the rolling becomes smooth.
Fig. 1 is a schematic view of an embodiment of a rolling machine according to the present invention;
Fig. 2 is an enlarged view of an important portion of the embodiment;
Fig. 3 is a perspective view of a pinch roll with projections of the embodiment;
Fig. 4 is a perspective view of a band plate formed with recesses; and
Fig. 5 is a graph showing the relationship between the rolling load and the reduction ratio.

The present invention will now be described in greater detail.

Fig. 1 is a schematic view of a rolling machine according to a preferred embodiment of the present invention, and Fig. 2 is an enlarged view of an important portion of the rolling machine. As shown in these drawings, the rolling machine 10 comprises a rolling mill 11 for rolling a band plate M, and a recess impressing unit 13 for forming recesses 12 in both sides of the band plate M on the inlet side of the rolling mill 11.

The rolling mill 11 includes upper and lower work rolls 14 and 15 for rolling the band plate M, and backup rolls 16 and 17 rotatable in contact with the upper and lower work rolls 14 and 15 to bear the reaction thereof, these individual rolls being rotatably supported by a housing 18.

Nozzles 19 and 20 are provided on the inlet side of the band plate M in relation to the work rolls 14 and 15 to spray a lubricating fluid L to individual contacting portions of the band plate M with the work rolls 14 and 15.

The recess impressing unit 13 provided on the upstream side of the rolling mill 11 includes a pair of projection-provided pinch rolls 22 and 23 having a large number of projections 21 as shown in Fig. 3, these pinch rolls being rotatably supported by a housing 24 so as to pinch the band plate M being fed.

It should be noted that the curvature of the recess 12 formed by the projection 21 is made larger than that of the work roll 14, but the shape of the recess 12 may take any form if it can be pressed completely flat at the time of rolling.

Further, the pinch rolls 22 and 23 pinch the band plate M at a pressure enough for the recess 12 to be formed by the corresponding projection 21 by virtue of the plastic deformation of the band plate M being fed.

Accordingly, when the band plate M is fed rightward in Fig. 1, at first, a large number of recesses 12 are formed in both sides of the band plate M by the recess impressing unit 13 as shown in Fig. 4. Then, when the band plate M formed with the recesses 12 is fed to the rolling mill 11, the fluid L sprayed to the contacting portions between the work rolls 14 and 15 and the band plate M is retained in the recesses 12 before being caught in the contacting arc regions α of the work rolls 14 and 15. Thereafter, at the time of the band plate M being rolled, the lubricating fluid L in the recesses 12 is temporarily confined in the recesses 12 because the surfaces of the work rolls 14 and 15 contact with the opening margins of the recesses 12. On the other hand, the fluid adhering to the surfaces of the work rolls 14 and 15 is introduced into the recesses 12 as the work rolls 14 and 15 rotate. Then, when the rolling progresses, the fluid L confined in the recesses 12 forms a boundary film over the contacting portions between the work rolls 14 and 15 and the band plate M because the recesses 12 are gradually expanded thin and flat within the contacting arc region. Since due to the formation of the boundary film the fluid L largely remains in the contacting arc region at the time of the band plate M being rolled in contrast with the prior art, the abrasion of the roll is reduced.

Further, since a large number of recesses 12 are formed in the band plate M, the amount of the fluid L being sprayed is sufficient if it is confined in the recesses 12 to remain therein enough, thus, the consumption of the fluid L can be decreased remarkably compared with the prior art.

Although the foregoing embodiment uses the projection-provided pinch rolls 22 and 23 to form the recesses 12 wherein the plastic working is attained through rolling, the recesses 12 may be formed through pressing or cutting.

Here, considering the reduction of the coefficient of friction between the work roll and the band plate according to the present invention, a general expression of the frictional shearing stress τ will be given below.

${\text{τ = aτ}}_{\text{b}} {\text{+ ( 1 - a ) τ}}_{\text{f}}$

where ${\text{τ}}_{\text{b}} \text{(=µP)}$ boundary friction zone,${\text{τ}}_{\text{f}} \text{(=η} \frac{\text{∂u}}{\text{∂h}} \text{)}$ is a fluid friction zone, µ is the coefficient of boundary friction, P is the bearing pressure of the roll, η is the viscosity of the fluid, u is the speed of the fluid, h is the thickness of the fluid, and a is the area ratio of the boundary friction zone.

Generally, µ= 0.2 to 0.5, and ${\text{τ}}_{\text{b}} {\text{»τ}}_{\text{f}}$ . Therefore, the frictional shearing stress τ can be decreased if the area ratio a is decreased.

That is, according to the present invention, to decrease the area ratio a, a large number of recesses 12 are formed in the surface of the band plate M before rolling, and the rolling is performed while confining the fluid L in the recesses 12. Therefore, the value of the area ratio a can be arbitrarily controlled by confining the fluid L in the recesses 12 formed in the band plate M.

Further, compared with the prior art, the fluid lubrication effect can be enhanced only by confining a small amount of fluid L in the recesses 12.

As the lubricating fluid used in the present invention, there is water.

As described above, the present invention can reduce the coefficient of friction in cold rolling of the band plate M.

Test performed will be described below to show the effectiveness of the present invention.

In the test, the band plate was an Al plate of 10mm thick, which was rolled at room temperature using a rolling mill having work rolls of 200mm diameter.

The lubricating agent was water, and the Al plate was machined to have recesses of 3mm diameter arranged at a pitch of 3mm.

A reference workpiece was an Al plate having no recess, which was similarly subjected to testing.

Fig. 5 shows the result of the test. As shown in Fig. 5, the rolling load was reduced in accordance with the present invention by about 20% to 40% compared with the reference workpiece having no recess, this exhibiting the effectiveness of the present invention.

Therefore, according to the present invention, the rolling load can be significantly reduced compared with the prior art; consequently, the individual components of the rolling mill, such as the backup rolls and housing for supporting the work rolls, can be made compact, allowing the rolling mill to be manufactured at low costs.

As described in detail with reference to the embodiment and the test, the present invention can reduce the coefficient of friction of the workpiece at the time of rolling and provide a large reduction ratio even if the rolling load is kept very small. Further, the surface roughness and abrasion of the rolling roll are reduced, the fluid serves effectively as an adiabatic agent, and the heat resistance of the roll is enhanced. In addition, with the rolling load reduced, the rolling mill can be made compact.

## Claims

1. A rolling method for rolling metal plates, metal bars or the like, where a large number of recesses (12) in the surface of a workpiece (M) to be rolled is formed,
characterized in that it is a cold rolling process where a lubricating fluid (L) being water is confined in the recesses (12) immediately prior to rolling the workpiece (M).

2. A rolling machine with a recess impressing unit (13) provided on the inlet side of a rolling mill (11) for rolling a workpiece (M), for forming in the surface of the workpiece (M) a large number of recesses (12) adapted for the retaining of a lubricating fluid (L) therein, and with at least one nozzle (19,20) for spraying the lubricating fluid (L),
characterized in that the nozzle (19, 20) provides water onto the workpiece (11) at the inlet side of work rolls (14, 15), for rolling, and that the rolling machine is a cold rolling machine.

3. A rolling machine according to claim 2, wherein said recess impressing unit (13) includes a pair of pinch rolls (22, 23) formed with a large number of projections (21).

## Patentansprüche

1. Walzverfahren zum Auswalzen von Metallplatten oder -blechen, Metallstangen o.dgl., wobei in der Oberfläche eines auszuwalzenden Werkstücks (M) eine große Zahl von Vertiefungen (12) ausgebildet werden, dadurch gekennzeichnet, daß es sich um einen Kaltwalzprozeß handelt, bei dem ein(e) Schmierfluid oder -flüssigkeit (L) in Form von Wasser unmittelbar vor dem Auswalzen des Werkstücks (M) in den Vertiefungen (12) eingeschlossen wird.

2. Walzmaschine mit einer an der Einlaufseite eines Walzwerks (11) zum Auswalzen eines Werkstücks (M) angeordneten Vertiefungsprägeeinheit (13), um in der Oberfläche des Werkstücks (M) eine große Zahl von Vertiefungen (12), welche darin ein(e) Schmierfluid oder -flüssigkeit (L) zu halten vermögen, auszubilden, und mit mindestens einer Düse (19, 20) zum Aufsprühen des (der) Schmierfluids bzw. -flüssigkeit (L), dadurch gekennzeichnet, daß die Düse (19, 20) an der Einlaufseite von Arbeitswalzen (14, 15) für das Auswalzen Wasser auf das Werkstück (M) liefert bzw. aufsprüht und daß die Walzmaschine eine Kaltwalzmaschine ist.

3. Walzmaschine nach Anspruch 2, wobei die Vertiefungsprägeeinheit (13) zwei Klemmwalzen (22, 23) aufweist, die jeweils mit einer großen Zahl von Vorsprüngen (21) versehen sind.

## Revendications

1. Procédé de laminage pour laminer des plaques métalliques, des barres métalliques ou des produits similaires, dans lequel on forme un grand nombre de creux (12) à la surface d'une pièce (M) à laminer, **caractérisé** en ce qu'il s'agit d'un processus de laminage à froid dans lequel le fluide de lubrification (L), qui est de l'eau, est confiné dans les creux (12) immédiatement avant le laminage de la pièce (M).

2. Machine de laminage avec une unité (13) d'impression de creux placée sur le côté d'entrée d'un train de laminage (11) pour laminer une pièce (M) afin de former à la surface de la pièce (M) un grand nombre de creux (12) aptes à retenir un fluide de lubrification (L), et avec au moins un injecteur (19, 20) pour projeter le fluide de lubrification (L), **caractérisée** en ce que l'injecteur (19, 20) envoie de l'eau sur la pièce (M) au niveau du côté d'entrée des cyliindres de travail (14, 15) du laminage et en ce que la machine de laminage est une machine de laminage à froid.

3. Machine de laminage selon la revendication 2, dans laquelle ladite unité (13) d'impression de creux inclut une paire de cylindres (22, 23) de pincement comportant un grand nombre de saillies (21).
